

W. F. M. McCARTY.  
PROCESS OF TREATING IRON AND STEEL.  
APPLICATION FILED NOV. 23, 1907.

901,362.

Patented Oct. 20, 1908.



Witnesses

J. Milton Fester.  
Myron S. Clear

William F. M. McCarty,

By P. L. Parker

Attorney

# UNITED STATES PATENT OFFICE.

WILLIAM F. MASON McCARTY, OF PLEASANTVILLE, NEW YORK, ASSIGNOR OF ONE-FOURTH TO GEORGE O. EATON, ONE-FOURTH TO THOMAS M. ACKEN, AND ONE-THIRTIETH TO ALEXANDER J. GUTTMAN, OF NEW YORK, N. Y.

## PROCESS OF TREATING IRON AND STEEL

No. 901,362.

Specification of Letters Patent. Patented Oct. 20, 1908.

Application filed November 28, 1907. Serial No. 403,452.

To all whom it may concern:

Be it known that I, WILLIAM F. MASON McCARTY, a citizen of the United States, residing at Pleasantville, in the county of 5 Westchester and State of New York, have invented certain new and useful Improvements in Processes of Treating Iron and Steel, of which the following is a specification:

10 This invention relates to processes of treating iron and steel, and particularly steel, to produce therefrom ingots which are free, or practically free, not only from sulfur and phosphorous but also from the occluded 15 or otherwise held gases which cause fissures, blow holes and like structural flaws in molded metal.

An important advantage of my invention resides in the fact that, in the practice of 20 my process, cyanogen, which exercises a highly deleterious effect upon steel, is practically wholly eliminated.

A further important advantage of my invention is that it is adapted to the treatment 25 of metals or ores containing titanium or metals of like character, which are injurious to steel.

In accomplishing the purposes of my invention I add to the materials from which 30 the metal is produced or to the metal after reduction, certain reagents which, by their reaction upon the impurities, under the conditions of the process as hereinafter set forth, effect the elimination thereof.

35 I have discovered that the contaminating impurities hereinbefore referred to, can be, to a great extent, removed by adding to the ore, or to the reduced metal, one or more chlorids decomposable at the temperature of molten iron, preferably a mixture of calcium chlorid ( $CaCl_2$ ) and sodium chlorid ( $NaCl$ ) and blowing superheated steam or superheated steam and air through the molten metal, or subjecting it, while in a 40 molten condition, to the action of a vacuum. I have also discovered that, by using the above mentioned reagents and blowing superheated steam or superheated steam and air through the molten metal, the impurities of the latter may be eliminated to an extent hitherto unobtainable, if such treatment is combined with or followed by the 45 subjection of the metal to the action of a vacuum.

In carrying out my process in its preferred form, I add to an average grade of ore or to the molten iron or steel therefrom, approximately 25 pounds of calcium chlorid and 100 pounds of sodium chlorid to every ton of metal or to the ores from which this 50 amount of metal may be reduced, the reduction of the ore being carried out in accordance with the usual practice in the art. The amount of chlorid or chlorids to be added depends upon the character of the ore or 55 metal treated. A determination of the nature and amount of impurities will enable a steel worker of some experience in using my process, to determine with fair accuracy just the amount of salts to be added. 70

If the metal has been produced in an ordinary blast-furnace it must be transferred to a Bessemer converter having a vacuum pump attachment of the character indicated in the accompanying drawing. It is advisable however to employ a blast furnace in which the metal may also be refined; such a furnace being illustrated in the drawing referred to. 75

After the addition of the calcium chlorid 80 and sodium chlorid, superheated steam is blown through the metal, preferably in rapidly occurring intermittent jets, or air and superheated steam are alternately passed through the liquid metal and the latter is 85 subjected to the action of a vacuum. The vacuum treatment may follow the injection of the steam or air and steam or the exhaust pump may be started when the steam or air and steam is turned on. The treatment with 90 steam and vacuum is continued until a test of the metal shows it to be freed from its impurities. A little experience in treating iron and steel from a certain source will render it possible to determine the proper duration 95 of the treatment with practical certainty.

While the conditions under which the reactions occur are such as to render it impossible to fully determine the exact chemical reactions which occur in the practice of my 100 process, it appears that the treatment with one or more chlorids and particularly chlorids of calcium and sodium, particularly where superheated steam is injected, causes a reaction of dissociated chlorin with the 105 sulfur, phosphorus and the difficultly removable gases in the metal, to produce therefrom gases, such for example, as, sulfur ox-

ids, hydrogen sulfid, hydrogen phosphid, chlorin sulfid and ammonia, which are not of a nature to be securely held by occlusion or otherwise in the molten metal, but may 5 be readily removed therefrom, particularly by the action of a vacuum. The treatment is particularly noteworthy in that cyanogen contained in the molten metal, is decomposed with the formation of ammonia, which is 10 particularly readily removed by the action of a vacuum. In treating metals or ores containing titanium or similar impurity, the latter forms compounds, with, it is thought, the chlorin and cyanogen present, which are 15 readily removed by volatilization from the material treated.

In the practice of my process I may advantageously employ the novel form of furnace shown in vertical section in the accompanying drawing, although my process may 20 be carried out practically and successfully, although not so advantageously, in other forms of furnaces or converters.

In the drawing 1 represents a furnace provided with a crucible 2 into which twyers 3 and 4 are arranged to discharge air and superheated steam respectively. Cocks 5 and 6 are provided to control the supply of air and steam. An outlet 7, adapted to be 25 closed by a fire clay plug is provided in the crucible 2.

The body of the furnace is provided throughout the greater portion of its length with double walls 8 and 9 as illustrated. 30 The inner wall depends from the upper solid portion of the furnace wall and terminates in an open lower end 10 which is of annular shape and of reduced diameter, the said end extending down into the crucible 2 to a point 35 below the level of the molten metal, which will be contained therein during the use of the furnace.

Between the inner and outer walls of the furnace is an annular chamber 11 which is 40 in communication with the crucible 2. The chamber 11 is connected with the interior of the furnace by numerous openings 12 arranged in the walls, above the melting zone. The furnace is supplied with a cover 13 45 which forms a substantially air tight joint with the top of the furnace.

Adjacent the top of the furnace I provide a pipe 14 which is connected with a powerful exhaust pump, (not shown) by which air 50 and the gases arising from the metal treated may be withdrawn, in the treatment of the metal as hereinbefore referred to. A brick-work support 15 may also be provided.

In the use of the furnace, in the preferred 55 practice of my process, it is charged with ore, flux and fuel, with the addition of calcium and sodium chlorids, before mentioned, and the charge treated in accordance with the usual practice in the operation of blast furnaces. When the ore has been reduced,

the metal in the crucible 2 is subjected to the treatment with superheated steam or air and superheated steam and the vacuum pump set in operation to withdraw air and gases through the pipe 14, as has been hereinbefore 70 fully described.

It will be noted that, inasmuch as the chamber 11 and openings 12 provide a passage for the steam or air and steam, which has passed through the metal in crucible 2, 75 it is not necessary to force or draw the entire body of steam or air and steam injected into the metal, through the mass remaining in the body of the furnace.

I have not claimed herein the furnace 80 which I have shown and described, as this invention will form the subject matter of a separate application which is now being prepared.

Metal treated by my process will be found 85 to be practically wholly free from impurities, to have a close fibrous or lamellar structure, be wholly free from fissures, flaws, seams, blow holes and the like, and to be possessed of great ductility, malleability and 90 tensile strength.

It is to be understood that known equivalents of the materials and steps hereinbefore recited may be employed without departing from the spirit of my invention or the scope 95 of the appended claims. It is also to be understood that the treated metal may, without departing from my process, be withdrawn from the furnace into a mold, by and under the action of a vacuum, as fully described in 100 my copending application for a method of producing ingots free from blowholes, filed July 12, 1907, Serial Number 382,488.

Having thus described my invention, I 105 claim:

1. A process of purifying iron and steel which consists in incorporating a chlorid therein and subjecting the metal, in a molten state, to the action of superheated steam.

2. A process of purifying iron and steel 110 which consists in incorporating sodium chlorid therein and subjecting the metal, in a molten state, to the action of superheated steam.

3. A process of purifying iron and steel 115 which consists in incorporating a chlorid therein, and subjecting the metal, in a molten state, to the action of superheated steam and a vacuum.

4. A process of purifying iron and steel 120 which consists in incorporating a chlorid therein and subjecting the metal, in a molten state, to the action of superheated steam, in intermittent jets or impulses and to the action of a vacuum.

5. A process of purifying iron and steel 125 which consists in incorporating sodium chlorid therein and subjecting the metal, in a molten state, to the action of superheated steam and a vacuum.

6. A process of purifying iron and steel which consists in incorporating sodium chlorid therein and subjecting the metal, in a molten state, to the action of superheated steam in intermittent jets or impulses and to the action of a vacuum.

7. A process of purifying iron and steel which consists in incorporating a chlorid therein, passing superheated steam through the metal, while in a molten state, and then subjecting it to the action of a vacuum.

8. A process of purifying iron and steel which consists in incorporating a chlorid therein, passing superheated steam in inter-  
15 mittent jets or impulses through the metal,

while in a molten state, and then subjecting it to the action of a vacuum.

9. A process of purifying iron and steel which consists in incorporating a chlorid therein, passing superheated steam and air 20 through the metal, while in a molten state, and then subjecting it to the action of a vacuum.

In testimony whereof I affix my signature in presence of two witnesses.

WILLIAM F. MASON MCCARTY.

Witnesses:

W. S. MOORE,  
LAURA R. AUSTIN.